

# UNITED STATES PATENT OFFICE.

CHARLES PANGBORN, OF KALAMAZOO, MICHIGAN.

## COMPOSITION OF MATTER FOR WELDING STEEL.

SPECIFICATION forming part of Letters Patent No. 700,979, dated May 27, 1902.

Application filed August 13, 1901. Serial No. 71,922. (No specimens.)

*To all whom it may concern:*

Be it known that I, CHARLES PANGBORN, a citizen of the United States, residing at Kalamazoo, in the county of Kalamazoo and State of Michigan, have invented a new and useful Composition of Matter to be Used for the Welding of Steel, of which the following is a specification.

My composition consists of the following ingredients, combined in the approximate proportions stated, viz: Iron chips, eighty-five pounds; boracic acid, fifteen pounds; gelatin, six ounces; water, one and one-fourth quarts. The gelatin is to be dissolved in the water by heating together and then added to the iron chips and thoroughly mixed. Then add the acid and mix thoroughly. (The gelatin is merely to make the acid adhere to the iron.)

By the use of the above compound steel can be welded as easily as iron.

I am aware that compositions have been used and patented containing borax and other ingredients for the same purpose; but I am not aware that boracic acid has ever been used for welding. A composition containing

borax when placed on hot steel crawls off, making it necessary to repeat the operation and requiring careful handling to prevent the compound from falling off, whereas by the use of boracic acid the compound adheres to the steel, even if the latter is placed in the fire in an inverted position, and with boracic acid steel welds at a lower heat than with borax, and thus lessens the chance of overheating the steel.

What I desire to secure by Letters Patent of the United States is—

1. Boracic acid combined with small particles of iron or steel for welding.
2. The combination of boracic acid, iron or steel, gelatin, and water, in the approximate proportions named above for a welding compound.

In testimony whereof I have signed my name to this specification in the presence of two subscribing witnesses.

CHARLES PANGBORN.

Witnesses:

JAMES I. VONDEFIFER,  
CORNELIUS BOODT.